



US008722299B2

(12) **United States Patent**  
**Sacripante et al.**

(10) **Patent No.:** **US 8,722,299 B2**  
(45) **Date of Patent:** **May 13, 2014**

(54) **CURABLE TONER COMPOSITIONS AND PROCESSES**

(75) Inventors: **Guerino G. Sacripante**, Oakville (CA); **Maria Jimena Loureiro**, Waterloo (CA); **Cuong Vong**, Hamilton (CA); **Richard P. N. Veregin**, Mississauga (CA); **Michael S. Hawkins**, Cambridge (CA); **Edward Graham Zwart**, Mississauga (CA)

(73) Assignee: **Xerox Corporation**, Norwalk, CT (US)

(\*) Notice: Subject to any disclaimer, the term of this patent is extended or adjusted under 35 U.S.C. 154(b) by 232 days.

(21) Appl. No.: **12/559,876**

(22) Filed: **Sep. 15, 2009**

(65) **Prior Publication Data**

US 2011/0065038 A1 Mar. 17, 2011

(51) **Int. Cl.**

**G03G 9/093** (2006.01)  
**G03G 9/087** (2006.01)

(52) **U.S. Cl.**

USPC ..... 430/110.2; 430/108.8; 430/109.4

(58) **Field of Classification Search**

USPC ..... 430/108.4, 108.8, 109.1, 110.1–110.3  
See application file for complete search history.

(56) **References Cited**

U.S. PATENT DOCUMENTS

|             |         |                  |
|-------------|---------|------------------|
| 3,590,000 A | 6/1971  | Palermi et al.   |
| 3,655,374 A | 4/1972  | Palermi et al.   |
| 3,720,617 A | 3/1973  | Chatterji et al. |
| 3,847,604 A | 11/1974 | Hagenbach et al. |
| 3,944,493 A | 3/1976  | Jadwin et al.    |

|             |         |                            |
|-------------|---------|----------------------------|
| 3,983,045 A | 9/1976  | Jugle et al.               |
| 4,007,293 A | 2/1977  | Mincer et al.              |
| 4,079,014 A | 3/1978  | Burness et al.             |
| 4,295,990 A | 10/1981 | Verbeek et al.             |
| 4,394,430 A | 7/1983  | Jadwin et al.              |
| 4,560,635 A | 12/1985 | Hoffend et al.             |
| 4,935,326 A | 6/1990  | Creatura et al.            |
| 4,937,166 A | 6/1990  | Creatura et al.            |
| 5,236,629 A | 8/1993  | Mahabadi et al.            |
| 5,278,020 A | 1/1994  | Grushkin et al.            |
| 5,290,654 A | 3/1994  | Sacripante et al.          |
| 5,302,486 A | 4/1994  | Patel et al.               |
| 5,308,734 A | 5/1994  | Sacripante et al.          |
| 5,330,874 A | 7/1994  | Mahabadi et al.            |
| 5,344,738 A | 9/1994  | Kmiecik-Lawrynowicz et al. |
| 5,346,797 A | 9/1994  | Kmiecik-Lawrynowicz et al. |
| 5,348,832 A | 9/1994  | Sacripante et al.          |
| 5,364,729 A | 11/1994 | Kmiecik-Lawrynowicz et al. |
| 5,366,841 A | 11/1994 | Patel et al.               |
| 5,370,963 A | 12/1994 | Patel et al.               |
| 5,403,693 A | 4/1995  | Patel et al.               |
| 5,405,728 A | 4/1995  | Hopper et al.              |
| 5,418,108 A | 5/1995  | Kmiecik-Lawrynowicz et al. |
| 5,496,676 A | 3/1996  | Croucher et al.            |
| 5,501,935 A | 3/1996  | Patel et al.               |

---

| (56)                  | References Cited |                            |                   |         |                                 |
|-----------------------|------------------|----------------------------|-------------------|---------|---------------------------------|
| U.S. PATENT DOCUMENTS |                  |                            |                   |         |                                 |
| 5,527,658 A           | 6/1996           | Hopper et al.              | 6,004,714 A       | 12/1999 | Ciccarelli et al.               |
| 5,585,215 A           | 12/1996          | Ong et al.                 | 6,063,827 A       | 5/2000  | Sacripante et al.               |
| 5,650,255 A           | 7/1997           | Ng et al.                  | 6,190,815 B1      | 2/2001  | Ciccarelli et al.               |
| 5,650,256 A           | 7/1997           | Veregin et al.             | 6,593,049 B1      | 7/2003  | Veregin et al.                  |
| 5,723,253 A           | 3/1998           | Higashino et al.           | 6,730,450 B1      | 5/2004  | Moffat et al.                   |
| 5,744,520 A           | 4/1998           | Kmiecik-Lawrynowicz et al. | 6,743,559 B2      | 6/2004  | Combes et al.                   |
| 5,747,215 A           | 5/1998           | Ong et al.                 | 6,756,176 B2      | 6/2004  | Stegamat et al.                 |
| 5,763,133 A           | 6/1998           | Ong et al.                 | 6,780,500 B2      | 8/2004  | Dumouchel                       |
| 5,766,818 A           | 6/1998           | Smith et al.               | 6,830,860 B2      | 12/2004 | Sacripante et al.               |
| 5,804,349 A           | 9/1998           | Ong et al.                 | 7,029,817 B2      | 4/2006  | Robinson et al.                 |
| 5,827,633 A           | 10/1998          | Ong et al.                 | 7,141,761 B1      | 11/2006 | Dirubio et al.                  |
| 5,840,462 A           | 11/1998          | Foucher et al.             | 7,749,673 B2 *    | 7/2010  | Zhou et al. .... 430/137.14     |
| 5,853,944 A           | 12/1998          | Foucher et al.             | 2005/0137278 A1 * | 6/2005  | Fromm et al. .... 522/100       |
| 5,863,698 A           | 1/1999           | Patel et al.               | 2006/0110674 A1   | 5/2006  | Maehata et al.                  |
| 5,869,215 A           | 2/1999           | Ong et al.                 | 2006/0216625 A1   | 9/2006  | Maehata et al.                  |
| 5,902,710 A           | 5/1999           | Ong et al.                 | 2006/0222991 A1   | 10/2006 | Sacripante et al.               |
| 5,910,387 A           | 6/1999           | Mychajlowskij et al.       | 2007/0122728 A1 * | 5/2007  | Vanbesien et al. .... 430/108.4 |
| 5,916,725 A           | 6/1999           | Patel et al.               | 2008/0095558 A1 * | 4/2008  | Schleusener .... 399/336        |
| 5,919,595 A           | 7/1999           | Mychajlowskij et al.       | 2008/0199797 A1 * | 8/2008  | Sacripante et al. .... 430/104  |
| 5,925,488 A           | 7/1999           | Patel et al.               | 2009/0035686 A1 * | 2/2009  | Sacripante .... 430/110.2       |
| 5,977,210 A           | 11/1999          | Patel et al.               | 2009/0047593 A1 * | 2/2009  | Vanbesien et al. .... 430/110.2 |
|                       |                  |                            | 2009/0220882 A1 * | 9/2009  | Zhou et al. .... 430/109.3      |
|                       |                  |                            | 2009/0246679 A1 * | 10/2009 | Nosella et al. .... 430/137.14  |
|                       |                  |                            | 2010/0055593 A1 * | 3/2010  | Zhou et al. .... 430/108.4      |

\* cited by examiner



FIG. 1



FIG. 2



FIG. 3



FIG. 4

**FIG. 5****FIG. 6**

## CURABLE TONER COMPOSITIONS AND PROCESSES

## BACKGROUND

This disclosure is generally directed to toner processes, and more specifically, emulsion aggregation and coalescence processes, as well as toner compositions formed by such processes and development processes using such toners.

Emulsion aggregation/coalescing processes for the preparation of toners are illustrated in a number of Xerox patents, such as U.S. Pat. Nos. 5,290,654, 5,278,020, 5,308,734, 5,370,963, 5,344,738, 5,403,693, 5,418,108, 5,364,729, and 5,346,797; and also of interest may be U.S. Pat. Nos. 5,348, 832; 5,405,728; 5,366,841; 5,496,676; 5,527,658; 5,585,215; 5,650,255; 5,650,256; 5,501,935; 5,723,253; 5,744,520; 5,763,133; 5,766,818; 5,747,215; 5,827,633; 5,853,944; 5,804,349; 5,840,462; 5,869,215; 5,863,698; 5,902,710; 5,910,387; 5,916,725; 5,919,595; 5,925,488 and 5,977,210.

Other patents disclosing exemplary emulsion aggregation/coalescing processes include, for example, U.S. Pat. Nos. 6,730,450, 6,743,559, 6,756,176, 6,780,500, 6,830,860, and 7,029,817.

The disclosures of each of the foregoing patents and publications are hereby incorporated by reference herein in their entirities. The appropriate components and process aspects of the each of the foregoing patents and publications may also be selected for the present compositions and processes in embodiments thereof.

Electrophotographic digital printing with conventional toners, including those of about 8 micron size, may result in very high pile heights for high surface coverage, for example, from about 12 microns to about 14 microns of height for surface area coverage of from about 300% to about 400%. When printed onto thin flexible packaging substrates, this large toner pile height may result in a wavy rewound roll. This wavy roll may be unusable for subsequent flexible packaging operations.

Thus, there remains a need for small size emulsion aggregation (EA) toners having a size of from about 3 microns to about 4 microns, which may be suitable for flexible packaging applications.

## SUMMARY

The present disclosure provides toners as well as processes for making such toners. In embodiments, a toner of the present disclosure may include a core including at least a first amorphous resin, optionally in combination with at least one crystalline resin, an optional colorant, and an optional wax; and a shell over at least a portion of the core including at least a second amorphous resin, wherein particles making up the toner are from about 2.5 microns to about 4.5 microns in diameter, wherein the second amorphous resin including the shell is present in an amount of from about 30 percent to about 40 percent by weight of the toner, and wherein the first amorphous resin and the second amorphous resin may be the same or different.

In embodiments, a toner of the present disclosure may include a core including at least a first amorphous polyester resin and a colorant, optionally in combination with at least one crystalline polyester resin and an optional wax; and a shell over at least a portion of the core including at least a second amorphous polyester resin, wherein particles making up the toner are from about 2.5 microns to about 4.5 microns in diameter, wherein the second amorphous polyester resin including the shell is present in an amount of from about 30

percent to about 40 percent by weight of the toner, and wherein the first amorphous polyester resin and the second amorphous polyester resin may be the same or different.

A process of the present disclosure may include, in embodiments, contacting an emulsion including a first amorphous polyester resin optionally in combination with a crystalline polyester resin, an optional wax, and an optional colorant to form particles; aggregating the particles; contacting the aggregated particles with at least a second amorphous polyester resin, optionally in combination with a photoinitiator, to form a shell over the aggregated particles; coalescing the aggregated particles to form toner particles; and recovering the toner particles, wherein particles making up the toner are from about 2.5 microns to about 4.5 microns in diameter, wherein the second amorphous resin including the shell is present in an amount of from about 30 percent to about 40 percent by weight of the toner, and wherein the first amorphous resin and the second amorphous resin may be the same or different.

## BRIEF DESCRIPTION OF THE DRAWINGS

Various embodiments of the present disclosure will be described herein below with reference to the figures wherein:

FIG. 1 is a graph depicting charge results for toners of the present disclosure and control toners having varying amounts of resin in the shell;

FIG. 2 is a graph depicting the effect the amount of resin in the shell had on charging characteristics of the toner;

FIG. 3 is a graph depicting charging characteristics of a cyan toner prepared in accordance with the present disclosure;

FIG. 4 is a graph depicting charging characteristics of a cyan toner prepared in accordance with the present disclosure; and

FIG. 5 is a graph depicting charging characteristics of a yellow toner prepared in accordance with the present disclosure; and

FIG. 6 is a graph depicting charging characteristics of a magenta toner prepared in accordance with the present disclosure.

## DETAILED DESCRIPTION

In accordance with the present disclosure, small particle sized low melt EA toners are provided which include a shell having more resin therein, and thus a greater thickness, compared with conventional toners having a core-shell configuration. These toners may be utilized in non-contact fusing applications.

In embodiments the present disclosure is directed to curable toner compositions, including those made by a chemical process such as emulsion aggregation, wherein the resultant toner composition includes an unsaturated polyester resin, optionally a wax, and optionally a colorant.

Processes of the present disclosure may include aggregating latex particles, such as latexes containing an unsaturated resin such as unsaturated crystalline or amorphous polymeric particles such as polyesters, optionally a wax, and optionally a colorant, in the presence of a coagulant. After particles are aggregated, a shell is applied thereto. The shell has a higher amount of resin compared with resins applied to conventional toners as a shell, and thus provides a shell with a greater thickness.

Low melting or ultra-low melting fixing temperatures can be obtained by the use of crystalline resins in the toner composition. The aforementioned low fixing temperatures allow

for the curing to occur at lower temperatures, such as from about 120° C. to about 135° C. The thicker shell minimizes migration of the pigment and crystalline resin to the surface of the particles, where the crystalline resin might otherwise reduce charging performance of the toner particles. The toner compositions provide other advantages, such as high temperature document offset properties, such as up to about 85° C., as well as increased pigment loading.

## Resin

Toners of the present disclosure may include any latex resin suitable for use in forming a toner. Such resins, in turn, may be made of any suitable monomer. Suitable monomers useful in forming the resin include, but are not limited to, acrylonitriles, diols, diacids, diamines, diesters, diisocyanates, combinations thereof, and the like. Any monomer employed may be selected depending upon the particular polymer to be utilized.

In embodiments, the polymer utilized to form the resin may be a polyester resin. Suitable polyester resins include, for example, sulfonated, non-sulfonated, crystalline, amorphous, combinations thereof, and the like. The polyester resins may be linear, branched, combinations thereof, and the like. Polyester resins may include, in embodiments, those resins described in U.S. Pat. Nos. 6,593,049 and 6,756,176, the disclosures of each of which are hereby incorporated by reference in their entirety. Suitable resins may also include a mixture of an amorphous polyester resin and a crystalline polyester resin as described in U.S. Pat. No. 6,830,860, the disclosure of which is hereby incorporated by reference in its entirety.

In embodiments, the resin may be a polyester resin formed by reacting a diol with a diacid or diester in the presence of an optional catalyst. For forming a crystalline polyester, suitable organic diols include aliphatic diols having from about 2 to about 36 carbon atoms, such as 1,2-ethanediol, 1,3-propanediol, 1,4-butanediol, 1,5-pantanediol, 1,6-hexanediol, 1,7-heptanediol, 1,8-octanediol, 1,9-nonanediol, 1,10-decanediol, 1,12-dodecanediol, ethylene glycol, combinations thereof, and the like. The aliphatic diol may be, for example, selected in an amount of from about 40 to about 60 mole percent, in embodiments from about 42 to about 55 mole percent, in embodiments from about 45 to about 53 mole percent of the resin.

Examples of organic diacids or diesters selected for the preparation of the crystalline resins include oxalic acid, succinic acid, glutaric acid, adipic acid, suberic acid, azelaic acid, fumaric acid, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid may be present, for example, in an amount from about 40 to about 60 mole percent of the resin, in embodiments from about 42 to about 55 mole percent of the resin, in embodiments from about 45 to about 53 mole percent.

Examples of crystalline resins include polyesters, polyamides, polyimides, polyolefins, polyethylene, polybutylene, polyisobutylene, ethylene-propylene copolymers, ethylene-vinyl acetate copolymers, polypropylene, mixtures thereof, and the like. Specific crystalline resins may be polyester based, such as poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-

sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copolymers(ethylene-adipate), poly(decylene-sebacate), poly(decylene-decanoate), poly(ethylene-decanoate), poly(ethylene-dodecanoate), poly(nonylene-sebacate), poly(nonylene-decanoate), copoly(ethylene-fumarate)-copolymers(ethylene-sebacate), copoly(ethylene-fumarate)-copolymers(ethylene-decanoate), copoly(ethylene-fumarate)-copolymers(ethylene-dodecanoate), and combinations thereof. The crystalline resin may be present, for example, in an amount of from about 5 to about 50 percent by weight of the toner components, in embodiments from about 10 to about 35 percent by weight of the toner components. The crystalline resin can possess various melting points of, for example, from about 30° C. to about 120° C., in embodiments from about 50° C. to about 90° C. The crystalline resin may have a number average molecular weight (Mn), as measured by gel permeation chromatography (GPC) of, for example, from about 1,000 to about 50,000, in embodiments from about 2,000 to about 25,000, and a weight average molecular weight (Mw) of, for example, from about 2,000 to about 100,000, in embodiments from about 3,000 to about 80,000, as determined by Gel Permeation Chromatography using polystyrene standards. The molecular weight distribution (Mw/Mn) of the crystalline resin may be, for example, from about 2 to about 6, in embodiments from about 3 to about 4.

Examples of diacid or diesters selected for the preparation of amorphous polyesters include dicarboxylic acids or diesters such as terephthalic acid, phthalic acid, isophthalic acid, fumaric acid, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid or diester may be present, for example, in an amount from about 40 to about 60 mole percent of the resin, in embodiments from about 42 to about 55 mole percent of the resin, in embodiments from about 45 to about 53 mole percent of the resin.

Examples of diols utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)bisphenol A, bis(2-hydroxypropyl)bisphenol A, 1,4-cyclohexanediethanol, 1,3-cyclohexanediethanol, xylenedimethanol, cyclohexanediol, diethylene glycol, bis(2-hydroxyethyl)oxide, dipropylene glycol, dibutylene, and combinations thereof. The amount of organic diol selected can vary, and may be present, for example, in an amount from about 40 to about 60 mole percent of the resin, in embodiments from about 42 to about 55 mole percent of the resin, in embodiments from about 45 to about 53 mole percent of the resin.

Polycondensation catalysts which may be utilized for either the crystalline or amorphous polyesters include tetraalkyl titanates, dialkyltin oxides such as dibutyltin oxide, tetraalkyltin oxides such as dibutyltin dilaurate, and dialkyltin oxide hydroxides such as butyltin oxide hydroxide, aluminum alkoxides, alkyl zinc, dialkyl zinc, zinc oxide, stannous oxide, or combinations thereof. Such catalysts may be utilized in amounts of, for example, from about 0.01 mole per-

cent to about 5 mole percent based on the starting diacid or diester used to generate the polyester resin.

In embodiments, suitable amorphous resins include polyesters, polyamides, polyimides, polyolefins, polyethylene, polybutylene, polyisobutylate, ethylene-propylene copolymers, ethylene-vinyl acetate copolymers, polypropylene, combinations thereof, and the like.

In embodiments, an unsaturated, amorphous polyester resin may be utilized as a latex resin. Examples of such resins include those disclosed in U.S. Pat. No. 6,063,827, the disclosure of which is hereby incorporated by reference in its entirety. Exemplary unsaturated amorphous polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof. In embodiments, the amorphous resin utilized in the core may be linear.

In embodiments, a suitable amorphous polyester resin may be a poly(propoxylated bisphenol A co-fumarate) resin having the following formula (I):



wherein m may be from about 5 to about 1000. Examples of such resins and processes for their production include those disclosed in U.S. Pat. No. 6,063,827, the disclosure of which is hereby incorporated by reference in its entirety.

An example of a linear propoxylated bisphenol A fumarate resin which may be utilized as a latex resin is available under the trade name SPARII from Resana S/A Industrias Quimicas, Sao Paulo Brazil. Other propoxylated bisphenol A polyester based resins that may be utilized and are commercially available include XP767, FXC42 and FXC-56 from Kao Corporation, Japan, and XP777 from Reichhold, Research Triangle Park, N.C., and the like.

In embodiments, a suitable amorphous resin utilized in a toner of the present disclosure may have a weight average molecular weight (Mw) of from about 10,000 to about 100,000, in embodiments from about 15,000 to about 30,000.

Suitable crystalline resins include those disclosed in U.S. Patent Application Publication No. 2006/0222991, the disclosure of which is hereby incorporated by reference in its entirety. In embodiments, a suitable crystalline resin may be composed of ethylene glycol and a mixture of dodecanedioic acid and fumaric acid co-monomers with the following formula:



wherein b is from about 5 to about 2000 and d is from about 5 to about 2000.

In embodiments, a suitable crystalline resin utilized in a toner of the present disclosure may have a molecular weight of from about 10,000 to about 100,000, in embodiments from about 15,000 to about 30,000.

One, two, or more resins may be used in forming a toner. In embodiments where two or more resins are used, the resins may be in any suitable ratio (e.g., weight ratio) such as, for instance, from about 1% (first resin)/99% (second resin) to about 99% (first resin)/1% (second resin), in embodiments from about 10% (first resin)/90% (second resin) to about 90% (first resin)/10% (second resin).

In embodiments, a suitable toner of the present disclosure may include 2 amorphous polyester resins and a crystalline polyester resin. The weight ratio of the three resins may be from about 29% first amorphous resin/69% second amorphous resin/2% crystalline resin, to about 60% first amorphous resin/20% second amorphous resin/20% crystalline resin.

As noted above, in embodiments, the resin may be formed by emulsion aggregation methods. Utilizing such methods, the resin may be present in a resin emulsion, which may then be combined with other components and additives to form a toner of the present disclosure.

The polymer resin may be present in an amount of from about 65 to about 95 percent by weight, or preferably from about 75 to about 85 percent by weight of the toner particles (that is, toner particles exclusive of external additives) on a solids basis. The ratio of crystalline resin to amorphous resin can be in the range from about 1:99 to about 30:70, such as from about 5:95 to about 25:75, in some embodiments from about 5:95 to about 15:95.

It has also been found that a polymer with a low acid number may be useful in forming toners. For example, it may be useful in embodiments that the acid number of the polymer is from about 0 to about 40 mg KOH/gram, such as from about 1 to about 30 mg KOH/gram, in embodiments from about 10 to about 20 mg KOH/gram.

Photoinitiator

In embodiments, where a polymer resin used to form a toner is unsaturated, it may be desirable to enhance curing of the unsaturated polymer by including an optional photoinitiator in the toner. Suitable photoinitiators include UV-photoinitiators including, but not limited to, hydroxycyclohexylphenyl ketones; other ketones such as alpha-amino ketone and

4-(2-hydroxyethoxy)phenyl-(2-hydroxy-2-propyl)ketone; benzoin; benzoin alkyl ethers; benzophenones, such as 2,4,6-trimethylbenzophenone and 4-methylbenzophenone; trimethylbenzoylphenylphosphine oxides such as 2,4,6-trimethylbenzoyl-diphenyl-phosphine oxide or phenylbis(2,4,6-trimethylbenzoyl)phosphine oxide (BAPO) available as IRGACURE® 819 from Ciba; azo compounds; anthraquinones and substituted anthraquinones, such as, for example, alkyl substituted or halo substituted anthraquinones; other substituted or unsubstituted polynuclear quinines; acetophenones, thioxanthones; ketals; acylphosphines; and mixtures thereof. Other examples of photoinitiators include,

but not limited to, 2-hydroxy-2-methyl-1-phenyl-propan-1-one and 2-isopropyl-9H-thioxanthen-9-one. In embodiments, the photoinitiator is one of the following compounds or a mixture thereof: a hydroxycyclohexylphenyl ketone, such as, for example, 2-Hydrox-4'-hydroxyethoxy-2-methyl-propiophenone or 1-hydroxycyclohexylphenyl ketone, such as, for example, IRGACURE® 184 (Ciba-Geigy Corp., Tarrytown, N.Y.), having the structure:



a trimethylbenzoylphenylphosphine oxide, such as, for example, ethyl-2,4,6-trimethylbenzoylphenylphosphinate, such as, for example, LUCIRIN® TPO-L (BASF Corp.), having the formula



a mixture of 2,4,6-trimethylbenzophenone and 4-methylbenzophenone, such as, for example, SARCURE™ SR1137 (Sartomer); a mixture of 2,4,6-trimethylbenzoyl-diphenylphosphine oxide and 2-hydroxy-2-methyl-1-phenyl-propan-1-one, such as, for example, DAROCUR® 4265 (Ciba Specialty Chemicals); alpha-amino ketone, such as, for example, IRGACURE® 379 (Ciba Specialty Chemicals); 4-(2-hydroxyethoxy)phenyl-(2-hydroxy-2-propyl) ketone, such as, for example, IRGACURE® 2959 (Ciba Specialty Chemicals); 2-isopropyl-9H-thioxanthen-9-one, such as, for example, DAROCUR® ITX (Ciba Specialty Chemicals); and mixtures thereof.

In embodiments, where a photoinitiator is utilized, the toner composition may contain from about 0.5 to about 15 wt % photoinitiator, such as a UV-photoinitiator, in embodiments from about 1 to about 14 wt %, or from about 3 to about 12 wt %, photoinitiator.

#### Toner

The resin of the resin emulsions described above, in embodiments a polyester resin, may be utilized to form toner compositions. Such toner compositions may include optional colorants, waxes, and other additives. Toners may be formed utilizing any method within the purview of those skilled in the art including, but not limited to, emulsion aggregation methods.

#### Surfactants

In embodiments, colorants, waxes, and other additives utilized to form toner compositions may be in dispersions including surfactants. Moreover, toner particles may be formed by emulsion aggregation methods where the resin and other components of the toner are placed in one or more surfactants, an emulsion is formed, toner particles are aggregated, coalesced, optionally washed and dried, and recovered.

One, two, or more surfactants may be utilized. The surfactants may be selected from ionic surfactants and nonionic surfactants. Anionic surfactants and cationic surfactants are encompassed by the term "ionic surfactants." In embodiments, the surfactant may be utilized so that it is present in an amount of from about 0.01% to about 5% by weight of the toner composition, for example from about 0.75% to about 4% by weight of the toner composition, in embodiments from about 1% to about 3% by weight of the toner composition.

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxaethylene nonylphenyl ether, dialkylphenoxy poly(ethyleneoxy)ethanol, available from Rhone-Poulenc as IGEPAL CA-210™, IGEPAL CA-520™, IGEPAL CA-720™, IGEPAL CO-890™, IGEPAL CO-720™, IGEPAL CO-290™, IGEPAL CA-210™, ANTAROX 890™ and ANTAROX 897™. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecyl naphthalene sulfate, dialkyl benzenealkyl sulfates and sulfonates, acids such as abitic acid available from Aldrich, NEOGEN R™, NEOGEN SCT™ obtained from Daiichi Kogyo Seiyaku, combinations thereof, and the like. Other suitable anionic surfactants include, in embodiments, DOWFAX™ 2A1, an alkyl diphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecylbenzyl triethyl ammonium chloride, MIRAPOL™ and ALKAQUAT™, available from Alkaril Chemical Company, SANIZOL™ (benzalkonium chloride), available from Kao Chemicals, and the like, and mixtures thereof.

#### Colorants

As the colorant to be added, various known suitable colorants, such as dyes, pigments, mixtures of dyes, mixtures of pigments, mixtures of dyes and pigments, and the like, may be included in the toner. The colorant may be included in the toner in an amount of, for example, about 3 to about 35 percent by weight of the toner, or from about 5 to about 20 weight percent of the toner, or from about 7 to about 15 percent by weight of the toner.

As examples of suitable colorants, mention may be made of carbon black like REGAL 330®; magnetites, such as Mobay magnetites MO8029™, MO8060™; Columbian magnetites; MAPICO BLACKSTM and surface treated magnetites; Pfizer magnetites CB4799™; CB5300™, CB5600™, MCX6369™; Bayer magnetites, BAYFERROX

8600<sup>TM</sup>, 8610<sup>TM</sup>; Northern Pigments magnetites, NP-604<sup>TM</sup>, NP-608<sup>TM</sup>; Magnox magnetites TMB-100<sup>TM</sup>, or TMB-104<sup>TM</sup>; and the like. As colored pigments, there can be selected cyan, magenta, yellow, red, green, brown, blue or mixtures thereof. Generally, cyan, magenta, or yellow pigments or dyes, or mixtures thereof, are used. The pigment or pigments are generally used as water based pigment dispersions.

Specific examples of pigments include SUNSPERSE 6000, FLEXIVERSE and AQUATONE water based pigment dispersions from SUN Chemicals, HELIOGEN BLUE L6900<sup>TM</sup>, D6840<sup>TM</sup>, D7080<sup>TM</sup>, D7020<sup>TM</sup>, PYLAM OIL BLUE<sup>TM</sup>, PYLAM OIL YELLOW<sup>TM</sup>, PIGMENT BLUE 1<sup>TM</sup> available from Paul Uhlich & Company, Inc., PIGMENT VIOLET 1<sup>TM</sup>, PIGMENT RED 48<sup>TM</sup>, LEMON CHROME YELLOW DCC 1026<sup>TM</sup>, E. D. TOLUIDINE RED<sup>TM</sup> and BON RED C<sup>TM</sup> available from Dominion Color Corporation, Ltd., Toronto, Ontario, NOVAPERM YELLOW FGL<sup>TM</sup>, HOSTAPERM PINK E<sup>TM</sup> from Hoechst, and CINQUASIA MAGENTA<sup>TM</sup> available from E.I. DuPont de Nemours & Company, and the like. Generally, colorants that can be selected are black, cyan, magenta, or yellow, and mixtures thereof. Examples of magentas are 2,9-dimethyl-substituted quinacridone and anthraquinone dye identified in the Color Index as CI 60710, CI Dispersed Red 15, diazo dye identified in the Color Index as CI 26050, CI Solvent Red 19, and the like. Illustrative examples of cyans include copper tetra(oc-tadecyl sulfonamido)phthalocyanine, x-copper phthalocyanine pigment listed in the Color Index as CI 74160, CI Pigment Blue, Pigment Blue 15:3, and Anthrathrene Blue, identified in the Color Index as CI 69810, Special Blue X-2137, and the like. Illustrative examples of yellows are diarylide yellow 3,3-dichlorobenzidine acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent Yellow FGL. Colored magnetites, such as mixtures of MAPICO BLACK<sup>TM</sup>, and cyan components may also be selected as colorants. Other known colorants can be selected, such as Levanyl Black A-SF (Miles, Bayer) and Sunperse Carbon Black LHD 9303 (Sun Chemicals), and colored dyes such as Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta (DuPont), Lithol Scarlet D3700 (BASF), Toluidine Red (Aldrich), Scarlet for Thermoplast NSD PS PA (Ugine Kuhlmann of Canada), E. D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing, and the like.

In embodiments, suitable colorants include Pigment Blue 15:3, black Pigment Regal 330, Black Pigment Nipex 35, Pigment Red 269, Pigment Red 122, Pigment Red 81:2, Pigment Yellow 74, Pigment Yellow 180, combinations thereof, and the like.

For conventional toners, a cyan pigment may be used in an amount from about 3.5% to about 5% for toners possessing particles having a diameter of from about 5 microns to about 7 microns; in accordance with the present disclosure, the cyan pigment may be present in an amount from about 5% to about 8% for toners possessing particles having a diameter of from about 2.5 microns to about 4.5 microns. For conventional toners, the black pigment may be present in an amount from about 5% to about 6% for toners possessing particles having a diameter of from about 5 microns to about 7 microns; in accordance with the present disclosure, the black pigment may be present in an amount from about 6% to about 10% for toners possessing particles having a diameter of from about 2.5 microns to about 4.5 microns. For conventional toners, the magenta pigment may be present in an amount from about 6% to about 10% for toners possessing particles having a diameter of from about 5 microns to about 7 microns; in accordance with the present disclosure, the magenta pigment may be present in an amount from about 8% to about 14% for toners possessing particles having a diameter of from about 2.5 microns to about 4.5 microns. For conventional toners, the yellow pigment may be present in an amount from about 6% to about 9% for toners possessing particles having a diameter of from about 5 microns to about 7 microns; in accordance with the present disclosure, the yellow pigment may be present in an amount from about 8% to about 12% for toners possessing particles having a diameter of from about 2.5 microns to about 4.5 microns.

#### Wax

In addition to the polymer binder resin, the toners of the present disclosure also optionally contain a wax, which can be either a single type of wax or a mixture of two or more different waxes. A single wax can be added to toner formulations, for example, to improve particular toner properties, such as toner particle shape, presence and amount of wax on the toner particle surface, charging and/or fusing characteristics, gloss, stripping, offset properties, and the like. Alternatively, a combination of waxes can be added to provide multiple properties to the toner composition.

Optionally, a wax may also be combined with the resin and UV additive in forming toner particles. When included, the wax may be present in an amount of, for example, from about 1 weight percent to about 25 weight percent of the toner particles, in embodiments from about 5 weight percent to about 20 weight percent of the toner particles.

Waxes that may be selected include waxes having, for example, a weight average molecular weight of from about 500 to about 20,000, in embodiments from about 1,000 to about 10,000. Waxes that may be used include, for example, polyolefins such as polyethylene, polypropylene, and polybutene waxes such as commercially available from Allied Chemical and Petrolite Corporation, for example POLYWAX<sup>TM</sup> polyethylene waxes from Baker Petrolite, wax emulsions available from Michaelman, Inc. and the Daniels Products Company, EPOLENE N-15<sup>TM</sup> commercially available from Eastman Chemical Products, Inc., and VISCOL 550-P<sup>TM</sup>, a low weight average molecular weight polypropylene available from Sanyo Kasei K. K.; plant-based waxes, such as carnauba wax, rice wax, candelilla wax, sumacs wax, and jojoba oil; animal-based waxes, such as beeswax; mineral-based waxes and petroleum-based waxes, such as montan wax, ozokerite, ceresin, paraffin wax, microcrystalline wax,

and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride distearate, and pentaerythritol tetra behenate; ester waxes obtained from higher fatty acid and multivalent alcohol multimers, such as diethyleneglycol monostearate, dipropyleneglycol distearate, diglyceryl distearate, and triglyceryl tetra stearate; sorbitan higher fatty acid ester waxes, such as sorbitan monostearate, and cholesterol higher fatty acid ester waxes, such as cholesteryl stearate. Examples of functionalized waxes that may be used include, for example, amines, amides, for example AQUA SUPERSLIP 6550<sup>TM</sup>, SUPER-SLIP 6530<sup>TM</sup> available from Micro Powder Inc., fluorinated waxes, for example POLYFLUO 190<sup>TM</sup>, POLYFLUO 200<sup>TM</sup>, POLYSILK 19<sup>TM</sup>, POLYSILK 14<sup>TM</sup> available from Micro Powder Inc., mixed fluorinated, amide waxes, for example MICROSPERSION 19<sup>TM</sup> also available from Micro Powder Inc., imides, esters, quaternary amines, carboxylic acids or acrylic polymer emulsion, for example JONCRYL 74<sup>TM</sup>, 89<sup>TM</sup>, 130<sup>TM</sup>, 537<sup>TM</sup>, and 538<sup>TM</sup>, all available from SC Johnson Wax, and chlorinated polypropylenes and polyethylenes available from Allied Chemical and Petrolite Corporation and SC Johnson wax. Mixtures and combinations of the foregoing waxes may also be used in embodiments. Waxes may be included as, for example, fuser roll release agents.

#### Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Pat. Nos. 5,290,654 and 5,302,486, the disclosures of each of which are hereby incorporated by reference in their entirety. In embodiments, toner compositions and toner particles may be prepared by aggregation and coalescence processes in which small-size resin particles are aggregated to the appropriate toner particle size and then coalesced to achieve the final toner-particle shape and morphology.

In embodiments, toner compositions may be prepared by emulsion-aggregation processes, such as a process that includes aggregating a mixture of an optional colorant, an optional wax and any other desired or required additives, and emulsions including the resins described above, optionally in surfactants as described above, and then coalescing the aggregate mixture. A mixture may be prepared by adding an optional wax or other materials, which may also be optionally in a dispersion(s) including a surfactant, to the emulsion, which may be a mixture of two or more emulsions containing the resin. The pH of the resulting mixture may be adjusted by an acid such as, for example, acetic acid, nitric acid or the like. In embodiments, the pH of the mixture may be adjusted to from about 2 to about 4.5. Additionally, in embodiments, the mixture may be homogenized. If the mixture is homogenized, homogenization may be accomplished by mixing at about 600 to about 4,000 revolutions per minute. Homogenization may be accomplished by any suitable means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a

divalent cation or a multivalent cation material. The aggregating agent may be, for example, polyaluminum halides such as polyaluminum chloride (PAC), or the corresponding bromide, fluoride, or iodide, polyaluminum silicates such as 5 polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxylate, calcium sulfate, magnesium acetate, magnesium nitrate, magnesium sulfate, zinc acetate, zinc nitrate, zinc sulfate, zinc chloride, 10 zinc bromide, magnesium bromide, copper chloride, copper sulfate, and combinations thereof. In embodiments, the aggregating agent may be added to the mixture at a temperature that is below the glass transition temperature (Tg) of the resin.

The aggregating agent may be added to the mixture utilized to form a toner in an amount of, for example, from about 0.1 parts per hundred (pph) to about 1 pph, in embodiments from about 0.25 pph to about 0.75 pph, in some embodiments about 20 0.5 pph. This provides a sufficient amount of agent for aggregation.

The gloss of a toner may be influenced by the amount of retained metal ion, such as Al<sup>3+</sup>, in the particle. The amount of retained metal ion may be further adjusted by the addition of EDTA. In embodiments, the amount of retained crosslinker, for example Al<sup>3+</sup>, in toner particles of the present disclosure may be from about 0.1 pph to about 1 pph, in embodiments from about 0.25 pph to about 0.8 pph, in embodiments about 0.5 pph.

In order to control aggregation and coalescence of the particles, in embodiments the aggregating agent may be metered into the mixture over time. For example, the agent may be metered into the mixture over a period of from about 30 to 25 about 240 minutes, in embodiments from about 30 to about 200 minutes. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from about 35° C. to about 70° C.

The particles may be permitted to aggregate until a predetermined desired particle size is obtained. A predetermined 45 desired size refers to the desired particle size to be obtained as determined prior to formation, and the particle size being monitored during the growth process until such particle size is reached. Samples may be taken during the growth process and analyzed, for example with a Coulter Counter, for average 50 particle size. The aggregation thus may proceed by maintaining the elevated temperature, or slowly raising the temperature to, for example, from about 40° C. to about 100° C., and holding the mixture at this temperature for a time from about 0.5 hours to about 6 hours, in embodiments from about hour 55 1 to about 5 hours, while maintaining stirring, to provide the aggregated particles. Once the predetermined desired particle size is reached, then the growth process is halted. In embodiments, the predetermined desired particle size is within the toner particle size ranges mentioned above.

The growth and shaping of the particles following addition 60 of the aggregation agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for example of from about 40° C. to about 90° C., in embodiments

## 13

ments from about 45° C. to about 80° C., which may be below the glass transition temperature of the resin as discussed above.

In embodiments, the aggregate particles may be of a size of less than about 3 microns, in embodiments from about 2 microns to about 3 microns, in embodiments from about 2.5 microns to about 2.9 microns.

## Shell Resin

In embodiments, a shell may be applied to the formed aggregated toner particles. Any resin described above as suitable for the core resin may be utilized as the shell resin. The shell resin may be applied to the aggregated particles by any method within the purview of those skilled in the art. In embodiments, the shell resin may be in an emulsion including any surfactant described above. The aggregated particles described above may be combined with said emulsion so that the resin forms a shell over the formed aggregates. In embodiments, an amorphous polyester may be utilized to form a shell over the aggregates to form toner particles having a core-shell configuration. In embodiments, an amorphous polyester of formula I above may be utilized to form a shell.

For previous toner particles, having a size of diameter of from about 4 to about 8 microns, and more specifically, for toners of from about 5 to about 7 microns, the optimal shell component may be about 26 to about 30% by weight of the toner particles, in some cases about 28% by weight.

In accordance with the present disclosure, it has been found that for smaller particles, possessing a diameter from about 2 to about 4 microns, a thicker shell may be desirable to provide excellent charging characteristics due to the higher surface area of the toner particle. Thus, the shell resin may be present in an amount of at least about 30 percent by weight of the toner, in embodiments from about 30 percent to about 40 percent by weight of the toner particles, in embodiments from about 32 percent to about 38 percent by weight of the toner particles, in embodiments from about 34 percent to about 36 percent by weight of the toner particles.

In embodiments a photoinitiator as described above may be included in the shell. Thus, the photoinitiator may be in the core, the shell, or both. The photoinitiator may be present in an amount of from about 1 percent to about 5 percent by weight of the toner particles, in embodiments from about 2 percent to about 4 percent by weight of the toner particles.

Emulsions including these resins may have a solids loading of from about 5% solids by weight to about 20% solids by weight, in embodiments from about 12% solids by weight to about 17% solids by weight, in embodiments about 13% solids by weight.

Once the desired final size of the toner particles is achieved, the pH of the mixture may be adjusted with a base to a value of from about 6 to about 10, and in embodiments from about 6.2 to about 7. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylene diamine tetraacetic acid (EDTA) may be added to help adjust the pH to the desired values noted above. The base may be added in amounts from about 2 to about 25 percent by weight of the mixture, in embodiments from about 4 to about 10 percent by weight of the mixture.

## Coalescence

Following aggregation to the desired particle size, with the formation of an optional shell as described above, the particles may then be coalesced to the desired final shape, the coalescence being achieved by, for example, heating the mix-

## 14

ture to a temperature of from about 55° C. to about 100° C., in embodiments from about 65° C. to about 75° C., in embodiments about 70° C., which may be below the melting point of the crystalline resin to prevent plasticization. Higher or lower temperatures may be used, it being understood that the temperature is a function of the resins used for the binder.

Coalescence may proceed and be accomplished over a period of from about 0.1 to about 9 hours, in embodiments from about 0.5 to about 4 hours.

After coalescence, the mixture may be cooled to room temperature, such as from about 20° C. to about 25° C. The cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freezedrying.

## Additives

In embodiments, the toner particles may also contain other optional additives, as desired or required. For example, the toner may include any known charge additives in amounts of from about 0.1 to about 10 weight percent, and in embodiments of from about 0.5 to about 7 weight percent of the toner. Examples of such charge additives include alkyl pyridinium halides, bisulfates, the charge control additives of U.S. Pat. Nos. 3,944,493, 4,007,293, 4,079,014, 4,394,430 and 4,560,635, the disclosures of each of which are hereby incorporated by reference in their entirety, negative charge enhancing additives like aluminum complexes, and the like.

Surface additives can be added to the toner compositions of the present disclosure after washing or drying. Examples of such surface additives include, for example, metal salts, metal salts of fatty acids, colloidal silicas, metal oxides, strontium titanates, mixtures thereof, and the like. Surface additives may be present in an amount of from about 0.1 to about 10 weight percent, and in embodiments of from about 0.5 to about 7 weight percent of the toner. Examples of such additives include those disclosed in U.S. Pat. Nos. 3,590,000, 3,720,617, 3,655,374 and 3,983,045, the disclosures of each of which are hereby incorporated by reference in their entirety. Other additives include zinc stearate and AEROSIL R972® available from Degussa. The coated silicas of U.S. Pat. Nos. 6,190,815 and 6,004,714, the disclosures of each of which are hereby incorporated by reference in their entirety, can also be present in an amount of from about 0.05 to about 5 percent, and in embodiments of from about 0.1 to about 2 percent of the toner, which additives can be added during the aggregation or blended into the formed toner product.

The characteristics of the toner particles may be determined by any suitable technique and apparatus. Volume average particle diameter  $D_{50v}$ , GSD<sub>v</sub>, and GSD<sub>n</sub> may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3. Toners produced in accordance with the present disclosure may possess excellent charging characteristics when exposed to extreme relative humidity (RH) conditions. The low-humidity zone (C zone) may be about 10° C./15% RH, while the high humidity zone (A zone) may be about 28° C./85% RH.

Toners of the present disclosure may also possess a toner charge (Q/D) of from about -2 mm to about -20 mm, in embodiments from about -4 mm to about -10 mm. Toners of

the present disclosure may possess a parent toner charge per mass ratio (Q/M) of from about -20  $\mu$ C/g to about -80  $\mu$ C/g, in embodiments from about -40  $\mu$ C/g to about -60  $\mu$ C/g.

Utilizing the methods of the present disclosure, desirable gloss levels may be obtained. Thus, for example, the gloss level of a toner of the present disclosure may have a gloss as measured by Gardner Gloss Units (ggu) of from about 20 ggu to about 100 ggu, in embodiments from about 50 ggu to about 95 ggu, in embodiments from about 60 ggu to about 90 ggu.

In embodiments, toners of the present disclosure may be utilized as ultra low melt (ULM) toners. In embodiments, the dry toner particles, exclusive of external surface additives, may have the following characteristics:

(1) Volume average diameter (also referred to as "volume average particle diameter") of from about 2.5 to 4.5 microns in diameter, in embodiments from about 3 to about 4.2 microns, in embodiments about 3.5 microns.

(2) Number Average Geometric Standard Deviation (GSDn) and/or Volume Average Geometric Standard Deviation (GSDv) of from about 1.18 to about 1.30, in embodiments from about 1.20 to about 1.25.

(3) Circularity of from about 0.9 to about 1 (measured with, for example, a Sysmex FPIA 2100 analyzer), in embodiments from about 0.95 to about 0.99, in other embodiments from about 0.96 to about 0.98.

(4) Glass transition temperature of from about 45° C. to about 60° C., in embodiments from about 48° C. to about 55° C.

(5) The toner particles can have a surface area, as measured by the well known BET method, of from about 1.3 to about 6.5  $\text{m}^2/\text{g}$ . For example, for cyan, yellow and black toner particles, the BET surface area can be less than 2  $\text{m}^2/\text{g}$ , such as from about 1.4 to about 1.8  $\text{m}^2/\text{g}$ , and for magenta toner, from about 1.4 to about 6.3  $\text{m}^2/\text{g}$ .

It may be desirable in embodiments that the toner particle possess separate crystalline polyester and wax melting points and amorphous polyester glass transition temperature as measured by DSC, and that the melting temperatures and glass transition temperature are not substantially depressed by plasticization of the amorphous or crystalline polyesters, or by the wax. To achieve non-plasticization, it may be desirable to carry out the emulsion aggregation at a coalescence temperature of less than the melting point of the crystalline component and wax components.

#### Developers

The toner particles thus formed may be formulated into a developer composition. The toner particles may be mixed with carrier particles to achieve a two-component developer composition. The toner concentration in the developer may be from about 1% to about 25% by weight of the total weight of the developer, in embodiments from about 2% to about 15% by weight of the total weight of the developer.

#### Carriers

Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of

styrene, methyl methacrylate, and/or silanes, such as triethoxy silane, tetrafluoroethylenes, other known coatings and the like. For example, coatings containing polyvinylidene-fluoride, available, for example, as KYNAR 301FTM, and/or polymethylmethacrylate, for example having a weight average molecular weight of from about 300,000 to about 350,000, such as commercially available from Soken, may be used. In embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t-butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100  $\mu\text{m}$  in size, in embodiments from about 50 to about 75  $\mu\text{m}$  in size, coated with about 0.5% to about 10% by weight, in embodiments from about 0.7% to about 5% by weight of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

#### Imaging

The toners can be utilized for electrophotographic processes, including those disclosed in U.S. Pat. No. 4,295,990, the disclosure of which is hereby incorporated by reference in its entirety. In embodiments, any known type of image development system may be used in an image developing device, including, for example, magnetic brush development, jumping single-component development, hybrid scavengelss development (HSD), and the like. These and similar development systems are within the purview of those skilled in the art.

Imaging processes include, for example, preparing an image with an electrophotographic device including a charging component, an imaging component, a photoconductive component, a developing component, a transfer component,

and a fusing component. In embodiments, the development component may include a developer prepared by mixing a carrier with a toner composition described herein. The electrophotographic device may include a high speed printer, a black and white high speed printer, a color printer, and the like.

Exemplary apparatuses for producing these images may include, in embodiments, a heating device possessing heating elements, an optional contact fuser, a non-contact fuser such as a radiant fuser, an optional substrate pre-heater, an image bearing member pre-heater, and a transfuser. Examples of such apparatus include those disclosed in U.S. Pat. No. 7,141,761, the disclosure of which is hereby incorporated by reference in its entirety.

Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser roll member. Fuser roll members are contact fusing devices that are within the purview of those skilled in the art, in which heat and pressure from the roll may be used to fuse the toner to the image-receiving medium. In embodiments, the fuser member may be heated to a temperature above the fusing temperature of the toner, for example to temperatures of from about 70° C. to about 160° C., in embodiments from about 80° C. to about 150° C., in other embodiments from about 90° C. to about 140° C., after or during melting onto the image receiving substrate.

In embodiments, the fusing of the toner image can be conducted by any conventional means, such as combined heat and pressure fusing such as by the use of heated pressure rollers. Such fusing steps can include an irradiation step, such as an ultraviolet irradiation step, for activating any photoinitiator that may be present, thereby causing crosslinking or curing of the unsaturated polymer contained in the toner composition. This irradiation step can be conducted, for example, in the same fusing housing and/or step where conventional fusing is conducted, or it can be conducted in a separate irradiation fusing mechanism and/or step. In some embodiments, this irradiation step may provide non-contact fusing of the toner, so that conventional pressure fusing may not be required.

For example, in embodiments, the irradiation can be conducted in the same fusing housing and/or step where conventional fusing is conducted. In embodiments, the irradiation fusing can be conducted substantially simultaneously with conventional fusing, such as by locating an irradiation source immediately before or immediately after a heated pressure roll assembly. Desirably, such irradiation is located immediately after the heated pressure roll assembly, such that crosslinking occurs in the already fused image.

In other embodiments, the irradiation can be conducted in a separate fusing housing and/or step from a conventional fusing housing and/or step. For example, the irradiation fusing can be conducted in a separate housing from the conventional such as heated pressure roll fusing. That is, the conventionally fused image can be transported to another development device, or another component within the same development device, to conduct the irradiation fusing. In this manner, the irradiation fusing can be conducted as an optional step, for example to irradiation cure images that require improved high temperature document offset properties, but not to irradiation cure images that do not require such improved high temperature document offset properties. The conventional fusing step thus provides acceptable fixed

image properties for moist applications, while the optional irradiation curing can be conducted for images that may be exposed to more rigorous or higher temperature environments.

5 In other embodiments, the toner image can be fused by irradiation and optional heat, without conventional pressure fusing. This may be referred to, in embodiments, as noncontact fusing. The irradiation fusing can be conducted by any suitable irradiation device, and under suitable parameters, to 10 cause the desired degree of crosslinking of the unsaturated polymer. Suitable non-contact fusing methods are within the purview of those skilled in the art and include, in embodiments, flash fusing, radiant fusing, and/or steam fusing.

In embodiments, the energy source for fusing can be 15 actinic, such as radiation having a wavelength in the ultraviolet or visible region of the spectrum, accelerated particles, such as electron beam radiation, thermal such as heat or infrared radiation, or the like. In embodiments, the energy may be actinic radiation. Suitable sources of actinic radiation 20 include, but are not limited to, mercury lamps, xenon lamps, carbon arc lamps, tungsten filament lamps, lasers, sunlight, and the like.

In other embodiments, non-contact fusing may occur by 25 exposing the toner to infrared light at a wavelength of from about 750 nm to about 4000 nm, in embodiments from about 900 to about 3000 nm, for a period of time of from about 20 milliseconds to about 4000 milliseconds, in embodiments from about 500 milliseconds to about 1500 milliseconds.

Where heat is also applied, the image can be fused by 30 irradiation such as by ultraviolet or infrared light, in a heated environment such as from about 100 to about 250° C., such as from about 125 to about 225° C. or from about 150 or about 160 to about 180 or about 190° C.

In embodiments, the toner image can be fused by cold 35 pressure fusing, i.e., without the application of heat. Fusing can be effected at any desired or effective nip pressure, in embodiments from about 500 pounds per square inch to about 10,000 pounds per square inch, in embodiments from about 1000 pounds per square inch to about 5,000 pounds per 40 square inch. One advantage with cold pressure fusing is that it requires low power, and unlike hot roll processes, no standby power. Thus, toners of the present disclosure may be utilized in systems that are more environmentally friendly, having lower energy requirements. Moreover, as heat is not 45 applied to the toners, the toners do not become molten and thus do not offset during fusing.

When the irradiation fusing is applied to the toner composition, the resultant fused image is provided with non document offset properties, that is, the image does not exhibit 50 document offset, at temperature up to about 90° C., such as up to about 85° C. or up to about 80° C. The resultant fused image also exhibits improved abrasion resistance and scratch resistance as compared to conventional fused toner images. Such improved abrasion and scratch resistance is beneficial, 55 for example, for use in producing book covers, mailers, and other applications where abrasion and scratches would reduce the visual appearance of the item. Improved resistance to solvents is also provided, which is also beneficial for such uses as mailers, and the like. These properties are particularly helpful, for example, for images that must withstand higher 60 temperature environments, such as automobile manuals that typically are exposed to high temperatures in glove compartments or printed packaging materials that must withstand heat sealing treatments.

65 In embodiments, UV radiation may be applied, either separately for fusing, or in combination with IR light as described above. Ultraviolet radiation, in embodiments from a medium

pressure mercury lamp with a high speed conveyor under UV light, such as about 20 to about 70 m/min., can be used, wherein the UV radiation is provided at a wavelength of from about 200 to about 500 nm for about less than one second. In embodiments, the speed of the high speed conveyor can be about 15 to about 35 m/min. under UV light at a wavelength of from about 200 to about 500 nm for about 10 to about 50 milliseconds (ms). The emission spectrum of the UV light source generally overlaps the absorption spectrum of the UV-initiator. Optional curing equipment includes, but is not limited to, a reflector to focus or diff-use the UV light, and a cooling system to remove heat from the UV light source. Of course, these parameters are exemplary only, and the embodiments are not limited thereto. Further, variations in the process can include such modifications as light source wavelengths, optional pre-heating, and the like.

Thus, light to be applied to fuse an image to a substrate may be from about 200 nm to about 4000 nm.

It is envisioned that the toners of the present disclosure may be used in any suitable procedure for forming an image with a toner, including in applications other than xerographic applications.

Utilizing the toners of the present disclosure, images may be formed on substrates, including flexible substrates, having a toner pile height of from about 1 micron to about 6 microns, in embodiments from about 2 microns to about 4.5 microns, in embodiments from about 2.5 to about 4.2 microns.

The following Examples are being submitted to illustrate embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 30° C.

## EXAMPLES

### Example 1

Preparation of an amorphous resin-photoinitiator emulsion including about 3% of phenylbis(2,4,6-trimethylbenzoyl) phosphine oxide photoinitiator and 97% of poly-(propoxylated bisphenol A-fumarate) available from Reichold as XP777 resin.

About 816 grams of ethyl acetate was added to about 125 grams of a poly(propoxylated bisphenol A co-fumarate) resin available from Reichold as XP777 resin. The resin was dissolved by heating to about 65° C. on a hot plate and stirring at about 200 rpm. About 100 grams of ethyl acetate was added to about 3.75 grams of phenylbis(2,4,6-trimethylbenzoyl) phosphine oxide (BAPO, available as IRGACURE 819) (3% by weight of resin). The BAPO was dissolved by heating to about 65° C. on a hot plate and stirring at about 200 rpm. Once both solutions had reached about 65° C., the BAPO solution was added to the resin solution.

In a separate 4 liter glass reactor vessel, about 3.05 grams (for an acid number of about 17) of sodium bicarbonate was added to about 708.33 grams of deionized water. This aqueous solution was heated to about 65° C. on a hot plate with stirring at about 200 rpm. The dissolved resin, BAPO, and ethyl acetate mixture was slowly poured into the 4 liter glass reactor containing this aqueous solution with homogenization at about 4,000 rpm. The homogenizer speed was then increased to about 10,000 rpm and left for about 30 minutes. The homogenized mixture was placed in a heat jacketed PYREX distillation apparatus, with stirring at about 200 rpm. The temperature was ramped up to about 80° C. at a rate of about 1° C./minute. The ethyl acetate was distilled from the mixture at about 80° C. for about 120 minutes. The mixture was cooled to below about 40° C. then screened through a 20 micron screen. The mixture was pH adjusted to about 7 using a 4% NaOH solution and centrifuged. The resulting resin included about 35.4% solids by weight in water, with particles having a volume average diameter of about 112 nanometers as measured with a HONEYWELL MICROTRAC® UPA150 particle size analyzer.

about 1° C./minute. The ethyl acetate was distilled from the mixture at about 80° C. for about 120 minutes. The mixture was cooled to below about 40° C. then screened through a 20 micron screen. The mixture was pH adjusted to about 7 using a 4% NaOH solution and centrifuged. The resulting resin included about 35.4% solids by weight in water, with particles having a volume average diameter of about 112 nanometers as measured with a HONEYWELL MICROTRAC® UPA150 particle size analyzer.

### Example 2

Preparation of an amorphous resin-photoinitiator emulsion including about 3% of phenylbis(2,4,6-trimethylbenzoyl) phosphine oxide photoinitiator and 97% of polyester resin, FXC42, available from Kao Corporation.

About 816 grams of ethyl acetate was added to about 125 grams of an amorphous polyester resin, commercially available as FXC42 resin, from Kao Corporation. The resin was dissolved by heating to about 65° C. on a hot plate and stirring at about 200 rpm. About 100 grams of ethyl acetate was added to about 3.75 grams of phenylbis(2,4,6-trimethylbenzoyl) phosphine oxide (BAPO, available as IRGACURE 819) (3% by weight of resin). The BAPO was dissolved by heating to about 65° C. on a hot plate and stirring at about 200 rpm. Once both solutions had reached about 65° C., the BAPO solution was added to the resin solution.

In a separate 4 liter glass reactor vessel, about 3.05 grams (for an acid number of about 17) of sodium bicarbonate was added to about 708.33 grams of deionized water. This aqueous solution was heated to about 65° C. on a hot plate with stirring at about 200 rpm. The dissolved resin, BAPO, and ethyl acetate mixture was slowly poured into the 4 liter glass reactor containing this aqueous solution with homogenization at about 4,000 rpm. The homogenizer speed was then increased to about 10,000 rpm and left for about 30 minutes. The homogenized mixture was placed in a heat jacketed PYREX distillation apparatus, with stirring at about 200 rpm. The temperature was ramped up to about 80° C. at a rate of about 1° C./minute. The ethyl acetate was distilled from the mixture at about 80° C. for about 120 minutes. The mixture was cooled to below about 40° C. then screened through a 20 micron screen. The mixture was pH adjusted to about 7 using a 4% NaOH solution and centrifuged. The resulting resin included about 35.2% solids by weight in water, with particles having a volume average diameter of about 130 nanometers as measured with a HONEYWELL MICROTRAC® UPA150 particle size analyzer.

### Example 3

Preparation of an amorphous resin-photoinitiator emulsion including about 3% of phenylbis(2,4,6-trimethylbenzoyl) phosphine oxide photoinitiator and 97% of polyester resin, FXC56, available from Kao Corporation.

About 816 grams of ethyl acetate was added to about 125 grams of a branched amorphous polyester resin, commercially available as FXC56 resin, from Kao Corporation. The resin was dissolved by heating to about 65° C. on a hot plate and stirring at about 200 rpm. About 100 grams of ethyl acetate was added to about 3.75 grams of phenylbis(2,4,6-trimethylbenzoyl)phosphine oxide (BAPO, available as IRGACURE 819) (3% by weight of resin). The BAPO was dissolved by heating to about 65° C. on a hot plate and stirring at about 200 rpm. Once both solutions had reached about 65° C., the BAPO solution was added to the resin solution.

21

In a separate 4 liter glass reactor vessel, about 3.05 grams (for an acid number of about 17) of sodium bicarbonate was added to about 708.33 grams of deionized water. This aqueous solution was heated to about 65° C. on a hot plate with stirring at about 200 rpm. The dissolved resin, BAPO, and ethyl acetate mixture was slowly poured into the 4 liter glass reactor containing this aqueous solution with homogenization at about 4,000 rpm. The homogenizer speed was then increased to about 10,000 rpm and left for about 30 minutes. The homogenized mixture was placed in a heat jacketed PYREX distillation apparatus, with stirring at about 200 rpm. The temperature was ramped up to about 80° C. at about 1° C./minute. The ethyl acetate was distilled from the mixture at about 80° C. for about 120 minutes. The mixture was cooled to below about 40° C. then screened through a 20 micron screen. The mixture was pH adjusted to about 7 using about 4% NaOH solution and centrifuged. The resulting resin included about 35.3% solids by weight in water, with particles having a volume average diameter of about 122 nanometers as measured with a HONEYWELL MICROTAC® UPA150 particle size analyzer.

## Example 4

Preparation of crystalline resin emulsion including a crystalline polyester resin, copoly(ethylene-dodecanoate)-co-poly-(ethylene-fumarate), derived from dodecanedioic acid, ethylene glycol and fumaric acid.

A one liter Parr reactor equipped with a heating mantle, mechanical stirrer, bottom drain valve and distillation apparatus was charged with dodecanedioic acid (about 443.6 grams), fumaric acid (about 18.6 grams), hydroquinone (about 0.2 grams), n-butylstannoic acid (FASCAT 4100) catalyst (about 0.7 grams), and ethylene glycol (about 248 grams). The materials were stirred and slowly heated to about 150° C. over about 1 hour under a stream of CO<sub>2</sub>. The temperature was then increased by about 15° C. and subsequently about 10° C. intervals, every 30 minutes, to about 180° C. During this time, water was distilled as a by product. The temperature was then increased by about 5° C. intervals over about a 1 hour period to about 195° C. The pressure was then reduced to about 0.03 mbar over about a 2 hour period and any excess glycols were collected in the distillation receiver. The resin was returned to atmospheric pressure under a stream of CO<sub>2</sub> and then trimellitic anhydride (about 12.3 grams) was added. The pressure was slowly reduced to about 0.03 mbar over about 10 minutes and held there for about another 40 minutes. The crystalline resin, copoly(ethylene-dodecanoate)-co-poly-(ethylene-fumarate), was returned to atmospheric pressure and then drained through the bottom drain valve to give a resin with a viscosity of about 87 Pa·s (measured at about 85° C.), an onset melting of about 69° C., melt point temperature peak of about 78° C., and recrystallization peak on cooling of about 56° C. as measured by the Dupont Differential Scanning Calorimeter. The acid value of the resin was found to be about 12 meq/KOH.

About 816 grams of ethyl acetate was added to about 125 grams of the above crystalline resin. The resin was dissolved by heating to about 65° C. on a hot plate and stirring at about 200 rpm. In a separate 4 liter glass reactor vessel was added about 4.3 grams of TAYCA POWER surfactant (from Tayca Corporation (Japan), a branched sodium dodecyl benzene sulfonate) (about 47% aqueous solution), about 2.2 grams of sodium bicarbonate (for acid number of approximately 12 meq/KOH) and about 708.33 grams of deionized water was added. This aqueous solution was heated to about 65° C. on a hot plate with stirring at about 200 rpm. The dissolved resin in ethyl acetate mixture was slowly poured into the 4 liter glass reactor containing the aqueous solution with homogenization at about 4,000 rpm. The homogenizer speed was then increased to about 10,000 rpm and left for about 30 minutes. The homogenized mixture was placed in a heat jacketed PYREX distillation apparatus, with stirring at about 200 rpm. The temperature was ramped up to about 80° C. at about 1° C./minute. The ethyl acetate

22

The dissolved resin in ethyl acetate mixture was slowly poured into the 4 liter glass reactor containing the aqueous solution with homogenization at about 4,000 rpm. The homogenizer speed was then increased to 10,000 rpm and left for about 30 minutes. The homogenized mixture was placed in a heat jacketed PYREX distillation apparatus, with stirring at about 200 rpm. The temperature was ramped up to about 80° C. at about 1° C./minute. The ethyl acetate was distilled from the mixture at about 80° C. for about 120 minutes. The mixture was cooled to below about 40° C. then screened through a 20 micron screen. The mixture was pH adjusted to about 7 using about 4% NaOH aqueous solution and centrifuged. The resulting resin included about 35.1% solids by weight in water, with a volume average diameter of about 108 nanometers as measured with a HONEYWELL MICROTAC® UPA150 particle size analyzer.

## Example 5

Preparation of a crystalline resin emulsion including a crystalline polyester resin, poly(nonane-dodecanoate), derived from dodecanedioic acid and 1,9-nanonediol.

A one liter Parr reactor equipped with a heating mantle, mechanical stirrer, bottom drain valve and distillation apparatus was charged with dodecanedioic acid (about 443.6 grams), 1,9-nanonediol (about 305 grams) and n-butylstannoic acid (FASCAT 4100) catalyst (about 0.7 grams). The materials were stirred and slowly heated to about 150° C. over about 1 hour under a stream of CO<sub>2</sub>. The temperature was then increased by about 15° C. and subsequently about 10° C. intervals, every 30 minutes to about 180° C. During this time, water was distilled as a by product. The temperature was then increased by about 5° C. intervals over about a 1 hour period to about 195° C. The pressure was then reduced to about 0.03 mbar over about a 2 hour period and any excess glycols were collected in the distillation receiver. The resin was returned to atmospheric pressure under a stream of CO<sub>2</sub> and then trimellitic anhydride (about 12.3 grams) was added. The pressure was slowly reduced to about 0.03 mbar over about 10 minutes and held there for about another 40 minutes. The crystalline resin, copoly(ethylene-dodecanoate)-co-poly-(ethylene-fumarate), was returned to atmospheric pressure and then drained through the bottom drain valve to give a resin with a viscosity of about 87 Pa·s (measured at about 85° C.), an onset melting of about 69° C., melt point temperature peak of about 78° C., and recrystallization peak on cooling of about 56° C. as measured by a Dupont Differential Scanning Calorimeter. The acid value of the resin was found to be about 12 meq/KOH.

About 816 grams of ethyl acetate was added to about 125 grams of the above crystalline resin and dissolved by heating to about 65° C. on a hot plate with stirring at about 200 rpm. In a separate 4 liter glass reactor vessel about 4.3 grams of TAYCA POWER surfactant (from Tayca Corporation (Japan), a branched sodium dodecyl benzene sulfonate) (about 47% aqueous solution), about 2.2 grams sodium bicarbonate (for acid number of approximately 12 meq/KOH), and about 708.33 grams of deionized water was added. This aqueous solution was heated to about 65° C. on a hot plate with stirring at about 200 rpm. The dissolved resin in ethyl acetate mixture was slowly poured into the 4 liter glass reactor containing the aqueous solution with homogenization at about 4,000 rpm. The homogenizer speed was then increased to about 10,000 rpm and left for about 30 minutes. The homogenized mixture was placed in a heat jacketed PYREX distillation apparatus, with stirring at about 200 rpm. The temperature was ramped up to about 80° C. at about 1° C./minute. The ethyl acetate

was distilled from the mixture at about 80° C. for about 120 minutes. The mixture was cooled to below about 40° C. then screened through a 20 micron screen. The mixture was pH adjusted to about 7 using about 4% NaOH aqueous solution and centrifuged. The resulting resin included about 10% solids by weight in water, with a volume average diameter of about 118 nanometers as measured with a HONEYWELL MICROTACR® UPA150 particle size analyzer.

## Examples 6-10

Black toner including about 37.8% of the amorphous resin of Example 2, about 37.8% of the amorphous resin of Example 3, about 6.7% of the crystalline resin of Example 5, about 8.7% carbon black pigment, and about 9% of a polyethylene wax available from IGI was prepared. The toner had about 26% shell coverage including the amorphous resin.

A 2 liter kettle was charged with about 104.5 grams of the polyester emulsion of Example 2, about 103.4 grams of the polyester emulsion of Example 3, about 33.2 grams of the crystalline polyester emulsion of Example 5, about 83.5 grams of Nipex 35 Pigment (16.75% solids), about 8.7 grams of Nipex 35 carbon black dispersion (about 17.42% solids), about 44.6 grams of a 13.5% aqueous emulsion of polyethylene wax available from IGI chemicals, about 522.7 grams of water, and about 3.1 grams of DOWFAX™ 2A1 surfactant (an alkylidiphenyloxide disulfonate from the Dow Chemical Company (about 46.75% aqueous solution)). The mixture was stirred at about 100 rpm. To this was then added about 0.3 M nitric acid solution, until a pH of 4.2 was achieved, followed by homogenizing at about 2,000 rpm. To this was then added aluminum sulfate (about 0.5 ppH), after which the homogenizer was increased to about 4200 rpm.

The mixture was then stirred at about 470 rpm with an overhead stirrer and placed in a heating mantle. The temperature was increased to about 32° C. over about a 30 minute period, during which period the particles grew to just over about 3  $\mu$ m.

The shell solution including about 55.8 grams of the polyester emulsion of Example 2 and about 55.2 grams of the polyester of Example 3, along with about 58.8 grams of water and about 2.2 grams of DOWFAX surfactant was pH adjusted using 0.3 M nitric acid to a pH of about 3.3. This was then added to the 2 liter kettle, when the particle size of the toner was about 2.9  $\mu$ m. The temperature was then increased in increments of 2° C. until a particle size of about 4.26  $\mu$ m was obtained, which occurred at around 38° C.

A solution including sodium hydroxide in water (about 4% by weight of NaOH) was added to freeze the size (prevent further growth) until the pH of the mixture was about 4. Following this, about 5.76 g of a chelating agent, EDTA (about 0.75 ppH), was added to remove the aluminum and the pH was further adjusted using 4% NaOH to obtain a pH of about 7.6. During these additions, the stirrer speed was gradually reduced to about 180 rpm. The mixture was then heated to about 80° C. over about 60 minutes, and further to about 89° C. over about 30 minutes. The pH was decreased to about 7 by drop wise addition of an aqueous buffer solution of sodium acetate and acetic acid (original buffer pH adjusted to about 5.9 with acetic acid to achieve desired buffer ratio). The mixture was set to coalesce at a temperature of about 89° C. and at a pH of about 7. The resulting toner particles were of spherical morphology and displayed a size of about 3.96  $\mu$ m with a GSD of about 1.21.

For Examples 7 to 10, toners including the same components and prepared by the same process of Example 6

described above were prepared, except that varying amounts of amorphous resin in the shell were utilized as set forth in Table below.

TABLE 1

| Toner ID   | Shell wt. % | Particle Size (V) | GSD (V) | Circularity |
|------------|-------------|-------------------|---------|-------------|
| Example 6  | 26%         | 3.96              | 1.21    | 0.979       |
| Example 7  | 28%         | 4.04              | 1.21    | 0.979       |
| Example 8  | 30%         | 3.92              | 1.19    | 0.962       |
| Example 9  | 32%         | 4.31              | 1.24    | 0.973       |
| Example 10 | 34%         | 3.92              | 1.19    | 0.971       |

## Examples 11-14

A cyan UV curable toner including about 46.5% of the amorphous resin-photoinitiator of Example 1, about 11.7% of the crystalline resin of Example 4 and about 7.8% Pigment Blue 15:3 was prepared. The toner had about 34% shell coverage including the amorphous resin-photoinitiator of Example 1.

A 4 liter kettle was charged with about 393.8 grams of the polyester-photoinitiator emulsion of Example 1, about 117.9 grams of the crystalline resin of Example 4, about 147 grams of cyan Pigment Blue 15:3 dispersion (about 23.5% solids available from Sun Chemicals), about 515.1 grams of water, and about 6.2 grams of DOWFAX™ 2A1 surfactant (an alkylidiphenyloxide disulfonate from the Dow Chemical Company (about 46.75% aqueous solution)). The mixture was stirred at about 100 rpm. To this was then added about 0.3 M nitric acid solution, until a pH of about 4.2 was achieved, followed by homogenizing at about 2,000 rpm. To this was then added aluminum sulfate (about 0.4 ppH), after which the homogenizer was increased to about 4200 rpm.

The mixture was then stirred at about 600 rpm with an overhead stirrer and placed in a heating mantle. The temperature was increased to about 30° C. over about a 30 minute period, during which period the particles grew to just below about 3  $\mu$ m.

A shell solution including about 289.6 grams of the polyester-photoinitiator from Example 1 in the above emulsion, along with about 265.2 grams of water and about 3.6 grams of DOWFAX surfactant was pH adjusted using about 0.3 M nitric acid to a pH of about 3.3. This was added to the 4 liter kettle when the particle size of the toner was about 2.9  $\mu$ m.

The temperature was then increased in increments of about 2° C. until a particle size of about 4.26  $\mu$ m was obtained, which occurred at around 42° C.

A solution including sodium hydroxide in water (about 4% by weight of NaOH) was added to freeze the size (prevent further growth) until the pH of the mixture was about 4. Following this, about 4.8 grams of a chelating agent, EDTA (about 0.75 ppH), was added to remove the aluminum and the pH was further adjusted using 4% NaOH to about 7.2. During these additions, the stirrer speed was gradually reduced to about 280 rpm.

The mixture was then heated to about 63° C. over about 60 minutes, and further to about 70° C. over about 30 minutes. The pH was decreased by increments of about 0.2 pH units by drop wise addition of an aqueous buffer solution of sodium acetate and acetic acid (original buffer pH adjusted to about 5.9 with acetic acid to achieve the desired buffer ratio). These pH changes occurred at about 44° C., about 50° C., about 56° C., about 62° C., and about 68° C. to reach a final pH of about 6.2. The mixture was set to coalesce at a temperature of about

70° C. and at a pH of about 6.2. The resulting toner particles were of spherical morphology and displayed a size of about 4.04  $\mu\text{m}$  with a GSD of about 1.21.

For Examples 12 to 14, a full color set of ultra-low melt ultraviolet curable toners were prepared utilizing the same procedure as described above for Example 11, with different pigments. These toners are summarized below in Table 2.

TABLE 2

| Toner ID   | Shell wt. % Pigment/Loading | Particle Size (V) | GSD (V) | GSD (N) | Circularity |
|------------|-----------------------------|-------------------|---------|---------|-------------|
| Example 11 | 34% Blue 15:3/7.8%          | 4.04              | 1.21    | 1.25    | 0.982       |
| Example 12 | 34% Black Nipex 35/8.7%     | 4.35              | 1.23    | 1.24    | 0.979       |
| Example 13 | 34% Yellow-74/9.4%          | 4.13              | 1.20    | 1.25    | 0.975       |
| Example 14 | 34% Red 81:2/11.5%          | 4.49              | 1.25    | 1.35    | 0.957       |

## Bench Q/D and Cohesion Results

Additive charge and cohesion data were obtained for these toners as follows.

Each toner sample was blended on a sample mill for about 30 seconds at about 15000 rpm. Developer samples were prepared with about 0.5 grams of each toner sample and about 10 grams of a ferrite carrier, and an additive design, sometimes referred to herein as additive package 1, which included including 0.88% by weight TiO<sub>2</sub> treated with a decylsilane (commercially available as JMT 2000 from Tayca), 1.73% by weight X24 (a sol-gel silica commercially available from Shin-Etsu Chemical), 0.55% by weight E10 (a cerium oxide commercially available from Mitsui Mining), 0.9% by weight Unilin 700 wax commercially available from Baker Petrolite, and about 1.71% by weight RY50 silica, a polydimethylsiloxane treated silica commercially available from Evonik Degussa, scaled proportionally for the smaller particle size.

A duplicate developer sample pair was prepared as above for each toner that was evaluated. One developer of the pair was conditioned overnight in A-zone (28° C./85% RH), and the other was conditioned overnight in the C-zone environmental chamber (10° C./15% RH). The next day, the developer samples were sealed and agitated for about 2 minutes, and then about 1 hour, using a Turbula mixer. After about 2 minutes and 1 hour of mixing, the triboelectric charge of the toner was measured using a charge spectrograph using a 100 V/cm field. The toner charge (Q/D) was measured visually as the midpoint of the toner charge distribution.

The charge was reported in millimeters of displacement from the zero line. Following the 1 hour of mixing, an additional 0.5 grams of toner sample was added to the already charged developer, and mixed for a further 15 seconds, where a Q/D displacement was again measured, and then mixed for a further 45 seconds (total 1 minute of mixing), and again a Q/D displacement was measured.

Considering the smaller particle size, all toner charge levels and charge distribution widths (indicated by “error” bars, admix, and RH sensitivity) were acceptable. All charge levels at 2 minutes (2') and 60 minutes (60') were close to the desired range of from about -4 mm to about -11 mm.

Charge results for the toners produced in Example 1, with varying amounts of resin in the shell, are summarized in FIG. 1 and FIG. 2. As can be seen in FIGS. 1 and 2, with lower amounts of shell, both the A-zone and C-zone charge were in the lower part of the desirable charge range. As the amount of resin in the shell increased, the A-zone initially decreased a slight amount, but then increased at the highest shell content. For the C-zone, charge increased with shell content. The highest shell concentration provided the highest overall

charge over all the zones, and thus provided a much better, centered, charge level in the desired charge space.

Charge results for the colored toners of Example 2 are summarized in FIGS. 3-6 (FIG. 3 was for the cyan toner, FIG. 4 was for the black toner, FIG. 5 was for the yellow toner, and FIG. 6 was for the magenta toner). The charge evaluation of the UV curable color toners set at 4 micron size, with 34% shell, resulted in an improvement in Q/d within the targets of -4 to -11, very comparable to a conventional toner that was 5.8 microns in size. Q/m in the C-zone was slightly high, but expected, due to the small size of these toners.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

## What is claimed is:

1. A toner consisting of: a core of at least a first amorphous resin, optionally in combination with at least one crystalline resin, and in combination with colorant of dyes, pigments, combinations of dyes, combination of pigments, and combinations of dyes and pigments in an amount of from about 0.1 to about 35 percent by weight of the toner, a wax selected from the group consisting of polyolefins, carnauba wax, rice wax, candelilla wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentylaerythritol tetra behenate, diethyleneglycol monostearate, dipropylene glycol distearate, diglyceryl distearate, triglyceryl tetrastearate, sorbitan monostearate, cholesteryl stearate, and combinations thereof, present in an amount of from about 1 weight percent to about 25 weight percent of toner, and a shell over at least a portion of the core of at least a second amorphous resin, wherein particles of the toner are from about 2.5 microns to about 4.5 microns in diameter and wherein the first amorphous resin and the second amorphous resin may be the same or different and wherein the second amorphous resin of the shell is an amorphous polyester of the formula:



wherein m may be from about 5 to about 1000 and wherein the shell second amorphous resin is present in an amount of from about 32 percent by weight of the toner to about 38 percent by weight of the toner.

2. The toner according to claim 1, wherein said at least one crystalline resin is present and is a polyester resin of the formula:



wherein  $b$  is from about 5 to about 2000 and  $d$  is from about 5 to about 2000.

3. The toner according to claim 1, wherein the colorant is carbon black and the wax is a polyolefin.

4. The toner according to claim 1, wherein the particles of the toner are from about 2.5 microns to about 4.2 microns in diameter.

5. The toner according to claim 1, wherein the toner possesses a parent toner charge per mass ratio of from about -20  $\mu\text{C/g}$  to about -80  $\mu\text{C/g}$ , a toner charge of from about -2 mm to about -20 mm, and wherein particles of the toner possesses a circularity of from about 0.95 to about 0.99.

6. A toner consisting of a photoinitiator, a core consisting of a first amorphous polyester resin in combination with a crystalline resin, a colorant, and a wax; and a shell over at least a portion of the core, said shell consisting of a second amorphous polyester resin, wherein particles of the toner are from about 2.5 microns to about 4.5 microns in diameter, wherein the first amorphous resin and the second amorphous resin may be the same or different, wherein said toner possesses a parent toner charge per mass ratio of from about -20  $\mu\text{C/g}$  to about -80  $\mu\text{C/g}$ , and a toner charge of from about -2 mm to about -20 mm, and wherein the second amorphous resin of the shell is an amorphous polyester of the formula:



wherein m may be from about 5 to about 1000 and wherein the shell second amorphous resin is present in an amount of from about 32 percent by weight of the toner to about 38 percent by weight of the toner.

7. A toner comprising: a core comprising at least a first amorphous resin and a colorant, optionally at least one crystalline polyester resin and a wax in combination with colorant of dyes, pigments, combinations of dyes, combination of pigments, and combinations of dyes and pigments in an amount of from about 0.1 to about 35 percent by weight of the toner, a wax selected from the group consisting of polyolefins, carnauba wax, rice wax, candelilla wax, sunacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentylerythritol tetra behenate, diethyleneglycol monostearate, dipropylene-glycol distearate, diglyceryl distearate, triglyceryl tetra stearate, sorbitan monostearate, cholesterlyl stearate, and combinations thereof, present in an amount of from about 1 weight

percent to about 25 weight percent of toner, and a shell over at least a portion of the core comprising at least a second amorphous polyester resin, wherein particles comprising the toner are from about 2.5 microns to about 4.5 microns in diameter, 5 wherein the second amorphous resin comprising the shell is present in an amount of from about 30 percent to about 40 percent by weight of the toner, wherein the first amorphous polyester resin and the second amorphous polyester resin may be the same or different and wherein the second amorphous resin of the shell is an amorphous polyester of the formula:



wherein m may be from about 5 to about 1000 and wherein the shell second amorphous resin is present in an amount of from about 32 percent by weight of the toner to about 38 percent by weight of the toner.

8. The toner according to claim 7, wherein the at least one crystalline polyester resin is present, is one and is of the formula:



wherein b is from about 5 to about 2000 and d is from about 5 to about 2000.

9. The toner according to claim 7, wherein the colorant is a pigment selected from the group consisting of Pigment Blue 15:3, black Pigment Regal 330, Black Pigment Nipex 35, Pigment Red 269, Pigment Red 122, Pigment Red 81:2, Pigment Yellow 74, Pigment Yellow 180, and combinations thereof in an amount of from about 0.1 to about 35 percent by weight of the toner and wherein the wax is selected from the group consisting of polyolefins, carnauba wax, rice wax, candillia wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentylaerythritol tetra behenate, diethyleneglycol monostearate, dipropylene glycol distearate, diglyceryl distearate, triglyceryl tetrastearate, and combinations thereof, present in an amount of from about 1 weight percent to about 25 weight percent of toner.

60 10. The toner according to claim 7, wherein the toner possesses a parent toner charge per mass ratio of from about -20  $\mu\text{C/g}$  to about -80  $\mu\text{C/g}$ , a toner charge of from about -2 mm to about -20 mm, and wherein particles of the toner possesses a circularity of from about 0.95 to about 0.99.

\* \* \* \*